

Jan. 30, 1968

J. E. BROWN ETAL

3,365,770

METHOD FOR MAKING STRETCH YARNS AND FABRICS

Filed June 26, 1964

2 Sheets-Sheet 1

FIG. 1



FIG. 3



FIG. 4

Inventors  
James E. Brown  
William Frank Taylor  
By their attorneys

*Hawson and Hawson*

Jan. 30, 1968

J. E. BROWN ET AL

3,365,770

METHOD FOR MAKING STRETCH YARNS AND FABRICS

Filed June 26, 1964

2 Sheets-Sheet 2



FIG. 2

Inventors  
James E. Brown  
William Frank Taylor  
By their attorneys  
Hawthorne and Hawthorne

3,365,770  
METHOD FOR MAKING STRETCH  
YARNS AND FABRICS

James E. Brown, Axis, and William Frank Taylor, Mobile, Ala., assignors to Courtaulds North America Inc., New York, N.Y., a corporation of Alabama

Filed June 26, 1964, Ser. No. 378,275

6 Claims. (Cl. 28—76)

This invention relates to a method for making stretch yarns and fabrics from cellulose filaments.

The use of stretchy yarns to make fabrics which have stretch properties has become increasingly widespread. Most of such yarns contain an elastomeric material, either as a component fiber or as an impregnant. The use of elastomers has drawbacks because in many instances they impart an undesirable hand or feel to the fabric and because they add to the cost of the fabric. Moreover, if stretch is imparted to the yarn before it is made into fabric, it becomes difficult to handle the yarn on conventional textile machinery.

There is therefore a need for an inexpensive yarn which will have stretch properties, and which can be processed on conventional textile machinery.

In accordance with the present invention, such yarns are made by treating a multi-ply yarn comprising at least 65% by weight cellulose filaments having a wet modulus of less than 1 g./denier at 5% extension with a swelling agent for cellulose equivalent in swelling effect to an aqueous solution containing between about 5 and about 40% NaOH, and between about 1 and about 8% NaCl, said yarn being treated in the substantial absence of tension, and then applying a reverse twist to the yarn.

Yarn made in accordance with the invention has an irregular appearance, as will be described more fully below. It may be drawn out and if retained in an extended position for a period of time, will lose its stretchy characteristics. In this condition it may be used on textile machinery like any non-stretch yarn, to make woven or knitted fabrics. Such fabrics upon being wetted out or steamed, without tension, will redevelop the stretch characteristics originally present in the yarn.

The invention therefore further includes a method for making a stretch fabric which comprises treating a multi-ply yarn comprising at least 65% by weight of regenerated cellulose filaments having a wet modulus not greater than 1 g./denier at 5% extension, with a swelling agent for cellulose equivalent to an aqueous solution containing between about 5 and about 40% by weight NaOH, and between about 1 and about 8% by weight NaCl, in the substantial absence of tension, to form a coiled yarn, reverse twisting the coiled yarn, extending the coiled, reverse twisted yarn to pull out the coils, converting the pulled out yarn to a fabric and relaxing the fabric in an aqueous fluid to develop stretch.

In its product aspects, the invention comprises a multi-ply stretchy yarn comprising at least 65% regenerated cellulose filaments having a wet modulus of less than 1 g./denier at 5% extension and having an irregular, three dimensional sequence of helical sections, the helix angle of succeeding sections varying in an arbitrary and random manner.

In the drawings:

FIGURE 1 is a flow diagram, illustrating the manufacture of stretch yarn in accordance with the invention.

FIG. 2 is a flow diagram illustrating the manufacture of stretch fabric in accordance with the invention.

FIG. 3 is a view in elevation of yarn which has been treated with swelling agent prior to reverse twisting.

FIG. 4 is a view in elevation of reverse twisted yarn made in accordance with the invention.

Referring to FIG. 1, yarn in accordance with the invention is made by treating a multi-ply yarn comprising at least 65% regenerated cellulose fiber or filaments having a wet modulus of 1 g./denier or less at 5% extension with a swelling agent equivalent to an aqueous solution containing 5 to 40% NaOH and 1 to 8% NaCl, in the absence of tension.

There are currently available on the open market several different types of regenerated cellulose. Conventional textile grade viscose rayon is characterized by a crenulated surface and a distinct skin-core structure. It may have a conditioned tenacity of say 2.0 to 4 g./denier and an elongation of say 14 to 30%. It is easily swollen in water and has a very low wet modulus, i.e., when wet a tension of not more than 1 g./denier is required to extend it 5%.

Another rayon currently available, though not ordinarily used in textiles, is the tire cord type. This, through the use of viscose modifiers, may have a smooth non-crenulated surface and no detectable skin-core structure. It may have a conditioned tenacity of 4-6 g./denier and an elongation of say 15 to 25%. Like conventional textile grade rayon, it too is easily swollen in water and has a wet modulus of less than 1 g./denier at 5% elongation.

Recently a new class of rayon has appeared on the market, variously known as "polynosique" or "high wet modulus" rayon. In general it is made by spinning unripened viscose into a bath low in regenerative power and then stretching to a high degree. See Tachikawa, 2,732,279, and Cox 2,937,070. Such rayons may have conditioned tenacities as high as 7-8 g./denier with extensibilities below 10%. They are characterized by wet moduli of above 1 g./denier at 5% extension.

In our copending application Ser. No. 363,248, filed Apr. 28, 1964, we have disclosed a method for making stretch yarns and fabrics in which a multi-ply cellulose yarn containing at least 65% high wet modulus rayon is subjected, while relaxed, to a swelling agent equivalent to an aqueous solution containing 5 to 40% NaOH. As pointed out in that application, solutions of this nature may be applied to high wet modulus rayon without adverse effect, but if applied to conventional rayon (or tire cord type rayon) they gelatinize it, breaking down the fiber structure. For this reason, cellulose fiber blends containing more than 35% textile grade rayon cannot be used with the process of my above copending application.

This is a substantial limitation on the use of the process described in said application since the cost of high wet modulus rayon is substantially higher than the cost of conventional rayon.

The present process meets this problem by employing a different class of swelling agents, namely those in which a modifying agent is employed to temper the action of the swelling agent. The preferred swelling agent for use in processes according to the present invention is an aqueous solution containing 5 to 40% NaOH and 1 to 8% NaCl. Equivalent solutions may, however, be made from various combinations of known cellulose swelling agents and salts. Thus, for example, the sodium hydroxide may be replaced by other alkali metal hydroxides and the sodium chloride by other alkali metal salts of strong mineral acids; or alkali metal salts of organic acids having ionization constants (20° C.) of 1.50 or greater.

The multi-ply yarn used in the invention has at least two plies and may have up to say 6 plies. The individual filaments making up the singles yarns may be staple filaments, or continuous filaments.

Yarns employed in the present invention may also include a minor proportion of non-cellulosic fibers, provided however that such fibers do not affect the basic nature of the blend.

The singles yarns used in the plied yarn may be of

any desired weight or construction varying from about 1 denier to about 15 denier. They may be twisted in either direction; and to any desired extent. The twist in the component singles yarns, should, however, be opposite in direction to the ply twist. Normally the singles yarns will have 10 to 40 turns per inch and the ply 5 to 40 turns per inch in the opposite direction.

The temperature at which the swelling agent is applied may be varied considerably. In accordance with well known principles, lower temperatures tend to cause a more vigorous swelling action. Conveniently, the treatment is carried out at room temperature (20° C. more or less) but may be carried out at any temperature between the freezing and boiling points of the solution.

The time of treatment will vary depending on the nature and concentration of the swelling agent and on the nature of the fiber, on the mechanical construction of the yarn and on mechanical details of the treating apparatus. Broadly, it may range from say 0.1 to 120 minutes.

The physical arrangements for treating the yarn may be any of those customarily used, provided that the yarn is maintained under substantially zero tension. The yarn may be passed through a bath of the swelling agent in the form of a catenary, or it may be laid down in a plaited pattern and passed through a bath, or sprayed, in that form. Alternatively, hanks or skeins may be passed through a bath or sprayed.

Following contact with the swelling agent, the yarn is washed, neutralized with acetic acid or some other relatively weak acid, and dried. All of these steps are carried out with the yarn under substantially zero tension.

At this stage the yarn is as shown in FIG. 3. It is composed of a helical series of regular coils, the coils being substantially contiguous with one another and having a helix angle approaching 90° (say more than 45°).

In accordance with the invention, the yarn is now reverse twisted, i.e., it is given a twist in a direction opposite to that in which it was plied. While the degree of reverse twist may vary, preferably it is between about 135 and 160% of the initial ply twist. The result is shown clearly in FIG. 4. As can be seen from the figure, the yarn is now an irregular three dimensional sequence of helical sections, the helix angle of succeeding sections varying in an arbitrary and random manner. The yarn is stretchy and when extended and released will recover its original length to a high degree.

It is difficult to process stretch yarn, as such, on looms and knitting machines; precisely because it is stretch yarn. However, this is not a problem with the present yarn because when the yarn is wound on a spool, preparatory to being converted into fabric, the tension incident to winding pulls the stretch out. If maintained under tension in the extended position for more than about 30 minutes, the yarn loses its recovery ability substantially entirely. Normally, the yarn stays wound on a spool for at least 24 hours before it is used and in this time the yarn loses its apparent stretchability. It can thus be woven or knitted just as though it had never had stretch characteristics. When, however, the resulting fabric is wetted, or steamed, under zero tension, the stretch characteristics redevelop and the result is a stretch fabric made of 100% cellulose. The steps required to make stretch fabric according to the invention are set out in FIG. 2.

The invention is illustrated in the following examples.

#### Example I

A 30/2 yarn is spun from 1½ denier 1¼" conventional rayon staple fiber having a wet modulus of about 0.3 g./denier at 5% elongation. The singles yarn has 30 turns per inch (t.p.i.) in the Z direction and is plied with 22.5 t.p.i. in the S direction. Samples are wound into skeins and treated for one minute at 20° C. in solutions as follows:

| Solution | NaOH | NaCl |
|----------|------|------|
| A        | 3    | 5    |
| B        | 4    | 5    |
| C        | 5    | 5    |
| D        | 7    | 5    |
| E        | 16   | 5    |
| F        | 20   | 5    |
| G        | 25   | 5    |

10 All samples are rinsed in water for 3 minutes at 150° F. They are then neutralized in 5% acetic acid, rinsed and dried at 250° F. The resulting yarns vary considerably in their stretchability, the maximum stretch being obtained with solution F.

#### Example II

A 24/2 yarn consisting of 100% textile grade rayon having a wet modulus of about 0.3 g./denier at 5% elongation is treated, in the skein, in the absence of tension with an aqueous solution containing 20% NaOH and 5% NaCl at 20° C. for 2 minutes. It is then washed, rinsed, neutralized with acetic acid, rinsed and dried (relaxed) at 120° C. The yarn is then reverse twisted 31.8 t.p.i. (148% of the ply twist). The yarn is wound into a skein and relaxed in water at 60° C. for 5 minutes. It is then extracted and dried, relaxed, at 120° C.

The yarn is then extended to maximum stretch, held for 5 minutes, relaxed for thirty seconds and the growth determined as

30 Percent growth =

$$\frac{\text{length after stretching} - \text{length before stretching}}{\text{length after stretching}} \times 100$$

35 From the growth, recovery is calculated as

Percent recovery =

$$\frac{\text{percent elongation} - \text{percent growth}}{\text{percent elongation}} \times 100$$

40 where

$$\text{Percent elongation} = \frac{\text{length at maximum stretch}}{\text{length before stretching}} \times 100$$

maximum stretch is found to be 167% with 59% recovery.

#### Example III

The reverse twisted yarn of Example II is spooled, pulling out the stretch. It is then woven as the filling, in a 46 x 34 fabric having an untreated rayon 8/1 warp yarns. After removal from the loom the fabric is desized and washed for 5 minutes at 88° C. for relaxation. The fabric is tumble dried. It is evaluated for stretch properties by ravelling a strip one inch wide and twelve inches long. Reference marks are placed at the ten inch point. The strip is then extended 25% and held for 5 minutes, relaxed for 5 minutes, again extended 25% and instantly relaxed. The recovery, calculated as above is found to be 69%.

60 What is claimed is:

1. A method of making a stretchy yarn which comprises contacting a multi-ply regenerated cellulose yarn at least 65% by weight of whose fibers have a wet modulus of not greater than 1 g./denier at 5% extension with a cellulose swelling agent equivalent to an aqueous solution of 5 to 40% sodium hydroxide and 1 to 8% NaCl, in the absence of tension, and then twisting the yarn in a direction opposite to its ply beyond the point where there is no twist in the original plied yarn.

70 2. The method claimed in claim 1 wherein the yarn is treated with an aqueous solution containing 5 to 40% NaOH at a temperature between about 0 and about 80° C. for between about 0.1 and about 120 minutes.

75 3. A method for making a stretch fabric which comprises treating a multi-ply yarn consisting essentially of

cellulose filaments having a wet modulus not greater than 1 g./denier at 5% extension with a swelling agent for cellulose equivalent to an aqueous solution containing between about 5 and about 40% NaOH and between about 1 and about 8% NaCl, at substantially zero tension, to form a coiled yarn, twisting the yarn in a direction opposite to its ply beyond the point where there is no twist in the original plied yarn, pulling out the coiled, reverse twisted yarn to form a substantially straight yarn, converting the straight yarn to a fabric and relaxing the fabric in an aqueous fluid.

4. The method claimed in claim 3 wherein the yarn is treated with an aqueous solution containing between

about 5 and about 40% NaOH, and between about 1 and about 8% NaCl, at a temperature between about 0° C. and about 80° C. for between about 0.1 and about 120 minutes.

5. A stretchy, multi-ply yarn produced according to the method of claim 1.

6. A stretch fabric produced according to the method of claim 3.

References Cited

UNITED STATES PATENTS

2,463,618 3/1949 Heberlein et al. ----- 57—157

JOHN PETRAKES, Primary Examiner.